

1

3,846,133

## MULTILAYERED COLOR PHOTOGRAPHIC MATERIAL WITH IMPROVED STABILITY UNDER TROPICAL CONDITIONS

Hugo Zorn, Munich-Lochhausen, Helmut Broll, Munich, and Erich Reckziegel, Leverkusen, Germany, assignors to Agfa-Gevaert Aktiengesellschaft, Leverkusen, Germany

No Drawing. Filed Oct. 4, 1972, Ser. No. 294,955  
Claims priority, application Germany, Oct. 6, 1971,

P 21 49 837.3

Int. Cl. G03c 1/76, 3/00

U.S. Cl. 96—74

3 Claims

### ABSTRACT OF THE DISCLOSURE

Stability to tropical conditions of color photographic multilayer materials comprising blue, green and red sensitive silver halide emulsion layers and color couplers therein, is improved if the red sensitized and/or the green sensitized silver halide emulsion layer contains colloidal silver.

This invention relates to a multilayered color photographic material whose stability under tropical conditions is improved by the addition of colloidal silver to at least one spectrally sensitized silver halide emulsion layer.

In order to enable photographic films to be stored under mild climatic conditions or at elevated temperatures, the necessary stability can be achieved by after-ripening the silver halide emulsions and by adding stabilizers such as mercapto compounds, organic disulfides, alkali metal thiosulfate complexes or triazaindolizines to the emulsions before casting the emulsions on a layer support. In many cases, particularly in color photographic films, these measures are not sufficient to ensure that the material will be stable when stored under tropical conditions with high humidities.

It has now been found that the stability of multilayered color photographic material against tropical conditions can be improved if at least one of the two silver halide emulsion layers which contain color-forming couplers and are sensitized to the red or green region of the spectrum respectively contains colloidal silver.

It is thought that this stabilizing effect is due to the colloidal silver protecting the sensitivity centres against the action of temperature and atmospheric moisture. In principle, any form of colloidal silver would have the effect required according to the invention but the yellow form dispersed in gelatin, so-called yellow silver, is preferred because it is almost completely transparent to red and green light and absorbs only blue light which is unwanted in the cyan-forming and magenta-forming layers. The blue sensitive yellow-forming layer, whose sensitivity would be reduced to a greater extent by the yellow silver, is in most cases much more resistant to tropical conditions than the cyan-forming and the magenta-forming layer and therefore generally, does not need stabilization with yellow silver. The quantities of colloidal silver to be added depend on the degree to which the stability under tropical conditions is required to be increased. In practice, it has been found that quantities of between 0.02 and 0.8 g. of colloidal silver per mol of silver halide are necessary in the emulsion to achieve the stabilizing effect. These quantities have little or no effect on the maximum reversal color density. The preparation of various types of colloidal silver has been described in the literature, e.g. in Weiser's "Colloidal Elements," Wiley & Sons, New York, 1933, which describes the preparation of yellow colloidal silver by the dextrin reduction method of Carey Lea, in German Pat. No. 1,096,193 (colloidal brown and black silver) and in U.S. Pat. No. 2,688,601 (colloidal blue silver).

2

The invention is explained with the aid of the following examples which demonstrate the colloidal silver of various forms is suitable for improving the stability under tropical conditions regardless of the nature of the emulsion, of the color coupler and of the method of color development, whether it be reversal development or negative development.

### EXAMPLE 1

Starting with a highly sensitive silver iodobromide emulsion which has been sensitized to the red region of the spectrum and which contains 5 mols percent of AgI, and 100 g. of 1-hydroxy-N-octadecyl-2-naphthamide per mol of silver halide as cyan-forming coupler three samples containing 0, 0.4 or 0.16 g. respectively of colloidal yellow silver per mol of silver halide were cast on a layer support of cellulose acetate. The silver content of the layer was 2 g./m.<sup>2</sup>. From each sample, an unexposed strip was stored for 7 days under conditions simulating a tropical climate, the temperature being 35° C. and the relative atmospheric humidity 85%. These strips and a corresponding strip of each sample which had not been stored in a tropical cupboard were exposed through a grey sensitometer wedge. The sample were developed by a process of color reversal development as follows:

(1) First development: 12 minutes at 24° C. in a thiocyanate-containing metol-hydroquinone developer of the following composition:

|                                       |      |     |
|---------------------------------------|------|-----|
| Sodium ethylene dianaminotetraacetate | g--  | 2   |
| p-N-monomethylaminophenol semisulfate | g--  | 4   |
| Sodium sulfite                        | g--  | 50  |
| Hydroquinone                          | g--  | 6   |
| Sodium carbonate                      | g--  | 35  |
| Sodium thiocyanate                    | g--  | 1.5 |
| Potassium bromide                     | g--  | 2   |
| Potassium iodide                      | g--  | 10  |
| Benzotriazole                         | mg-- | 250 |
| Made up with water to 1000 ml.        |      |     |
| pH 10.0±0.1.                          |      |     |

(2) Washing: 5 minutes.

(3) Second exposure: 1 minute.

(4) Reversal development: 15 minutes at 24° C. in a color developer of the following composition:

|                                                                                                     |      |    |
|-----------------------------------------------------------------------------------------------------|------|----|
| Nitrilotriacetic acid                                                                               | g--  | 2  |
| Sodium sulfite                                                                                      | g--  | 5  |
| Hydroxylamine sulfate                                                                               | g--  | 1  |
| Trisodium phosphate                                                                                 | g--  | 20 |
| Potassium bromide                                                                                   | g--  | 1  |
| Potassium iodide                                                                                    | mg-- | 10 |
| 4 - amino - 3 - methyl - N - ethyl - N - (β-methylsulfonamidoethyl)-anilinoesquisulfate monohydrate | g--  | 9  |
| 50% ethylene diamine                                                                                | ml-- | 6  |
| Made up with water to 1000 ml.                                                                      |      |    |
| pH 12.0.                                                                                            |      |    |

The samples were then treated by the usual methods of clarifying, bleaching the silver, fixing and washing. The developed strips were assessed in a Macbeth densitometer behind a red filter.

The following table shows the specific sensitivity

$$S_s = \log I \cdot t \text{ for the color density } \frac{D_{\max} + C_F}{2}$$

(C<sub>F</sub>=color fog at total exposure) and the maximum color density D<sub>max</sub> as well as the changes in these values ΔS<sub>s</sub>

and  $\Delta D_{max}$  observed after storage under tropical conditions.

TABLE 1

| G. of colloidal silver per mol of silver halide.....            | 0     | 0.04  | 0.16  |
|-----------------------------------------------------------------|-------|-------|-------|
| $S_s$ .....                                                     | 2.54  | 2.57  | 2.54  |
| $\Delta S_s$ (after storage under tropical conditions).....     | -0.30 | -0.23 | -0.19 |
| $D_{max}$ .....                                                 | 2.36  | 2.36  | 2.40  |
| $\Delta D_{max}$ (after storage under tropical conditions)..... | -0.20 | +0.07 | +0.06 |

It is clear from the figures that the losses in sensitivity and color density due to storage under tropical conditions are reduced by increasing quantities of colloidal silver yellow without the color reversal sensitivity  $S_s$  and the maximum color density  $D_{max}$  of the fresh material being suppressed.

## EXAMPLE 2

An emulsion layer which had been sensitized to the green region of the spectrum and contained 1-(2',4',6'-trichlorophenyl)-3-(m-pentadecylphenoxy carbamido)-pyrazolone-(5) as magenta-forming coupler was used instead of the cyan-forming layer used in Example 1. Four samples were prepared with increasing concentration of yellow colloidal silver and treated and assessed as described in Example 1. The measurements were carried out behind a green filter.

TABLE 2

| G. of colloidal silver per mol of silver halide..... | 0     | 0.04  | 0.16  | 0.64  |
|------------------------------------------------------|-------|-------|-------|-------|
| $S_s$ .....                                          | 2.37  | 2.34  | 2.33  | 2.47  |
| $\Delta S_s$ (after tropical storage).....           | -0.25 | -0.21 | -0.17 | -0.11 |
| $D_{max}$ .....                                      | 3.32  | 2.96  | 2.94  | 2.66  |
| $\Delta D_{max}$ (after tropical storage).....       | -0.02 | -0.05 | -0.02 | -0.01 |

This table again clearly shows the stabilizing effect of colloidal yellow silver. It reduces the maximum color density  $D_{max}$  of the fresh material to a slight extent but has no deleterious effect on the specific sensitivity  $S_s$ .

## EXAMPLE 3

The procedure is the same as that employed in Example 2 except that 20 g. of a white coupler of the formula 1-(4'-sulfophenyl)-3-heptadecyl-4-methyl-pyrazolone-(5) are added per kg. of emulsion in addition to 48 g. of the magenta-forming coupler previously mentioned.

TABLE 3

| G. of colloidal silver per mol of silver halide..... | 0     | 0.20  | 0.40  |
|------------------------------------------------------|-------|-------|-------|
| $S_s$ .....                                          | 2.84  | 2.72  | 2.66  |
| $\Delta S_s$ (after tropical storage).....           | -0.54 | -0.48 | -0.13 |
| $D_{max}$ .....                                      | 2.94  | 2.92  | 2.94  |
| $\Delta D_{max}$ (after tropical storage).....       | -0.16 | -0.22 | -0.20 |

## EXAMPLE 4

The procedure is the same as that employed in Example 1 except that a silver iodobromide emulsion of medium sensitivity containing 4 mol percent of AgI is used instead of the highly sensitive emulsion.

TABLE 4

| G. of colloidal silver per mol of silver halide..... | 0     | 0.20  | 0.40  | 0.60  |
|------------------------------------------------------|-------|-------|-------|-------|
| $S_s$ .....                                          | 2.30  | 2.31  | 2.24  | 2.16  |
| $\Delta S_s$ (after tropical storage).....           | -0.35 | -0.32 | -0.28 | -0.21 |
| $D_{max}$ .....                                      | 2.50  | 2.52  | 2.26  | 2.00  |
| $\Delta D_{max}$ (after tropical storage).....       | -0.55 | -0.72 | -0.52 | -0.30 |

## EXAMPLE 5

The procedure is the same as that employed in Example 4 with the exception that various types of colloidal silver are added to the medium sensitivity cyan-forming layer to improve the stability under tropical conditions. The materials are subjected once to a reversal development as in

the previous examples and once to a conventional color negative development using a color developer of the following composition:

|                                                                                                               |    |     |
|---------------------------------------------------------------------------------------------------------------|----|-----|
| Benzyl alcohol                                                                                                | ml | 4.2 |
| 5 Sodium hexametaphosphate                                                                                    | g  | 2   |
| Sodium sulfite anhydrous                                                                                      | g  | 2   |
| Potassium bromide                                                                                             | g  | 1.5 |
| Sodium metaborate cryst.                                                                                      | g  | 80  |
| 10 4 - amino - 3 - methyl - N - ethyl - N - (β - methylsulfonamido - ethyl) - anilinoesquisulfate monohydrate | g  | 5   |
| Made up with water to 1000 ml.                                                                                |    |     |
| pH 10.8±0.1.                                                                                                  |    |     |
| 15 Development temperature, 24° C.                                                                            |    |     |
| Development time, 12 minutes.                                                                                 |    |     |

The relative sensitivity  $S$  achieved in colour negative development is indicated in  $\log I \cdot t$  units measured at density 0.1 over the fog.

TABLE 5

| Nature of colloidal silver added                     | Colloidal yellow silver <sup>1</sup> | Grey brown <sup>2</sup> | Black <sup>3</sup> |
|------------------------------------------------------|--------------------------------------|-------------------------|--------------------|
| G. of colloidal silver per mol of silver halide..... | 0                                    | 0.60                    | 0.60               |
| Reversal development:                                |                                      |                         |                    |
| $S_s$ .....                                          | 2.30                                 | 2.19                    | 2.23               |
| $\Delta S_s$ (after tropical storage).....           | -0.30                                | +0.01                   | -0.16              |
| $D_{max}$ .....                                      | 2.18                                 | 1.84                    | 2.14               |
| $\Delta D_{max}$ (after tropical storage).....       | +0.11                                | -0.14                   | +0.01              |
| Colour negative development:                         |                                      |                         |                    |
| $S_s$ .....                                          | 3.40                                 | 3.30                    | 3.25               |
| $\Delta S$ (after tropical storage).....             | -0.42                                | +0.12                   | -0.27              |

<sup>1</sup> Prepared by Carey Lea method.

<sup>2</sup> According to D.B.P. No. 1,036,193, Example 1, but without blue black particles.

<sup>3</sup> According to D.B.P. No. 1,036,193, Example 1 (with blue black particles).

What is claimed is:

1. A color-photographic multilayer material having compounds that produce a negative image by imagewise exposure followed by developing treatment or reversal treatment producing positive image comprising at least one red-sensitized silver halide emulsion layer containing a cyan-forming coupler, at least one green-sensitized silver halide emulsion layer containing a magenta-forming coupler and at least one blue-sensitive silver halide emulsion layer containing a yellow-forming coupler, wherein the improvement comprises at least one of the emulsion layers of the group consisting of green-sensitized and red-sensitized emulsion layers comprises in the same phase a binder, a silver iodobromide colloidal silver and the color coupler.

2. A color-photographic material as claimed in claim 1 wherein said colloidal silver containing layer contains 0.02 to 0.8 g. of colloidal silver per mol of silver iodobromide.

3. A color-photographic material as claimed in claim 1 wherein the said colloidal silver containing layer contains a gelatin binder and a yellow colloidal silver.

## References Cited

## UNITED STATES PATENTS

|              |         |                 |         |
|--------------|---------|-----------------|---------|
| 60 2,673,800 | 3/1954  | Meeussen et al. | 96-74 X |
| 2,704,711    | 3/1955  | Hanson, Jr.     | 96-74 X |
| 2,875,052    | 2/1959  | Weyde           | 96-68   |
| 3,206,310    | 9/1965  | Herz            | 96-67   |
| 3,211,552    | 10/1965 | Chu             | 96-74   |

DAVID KLEIN, Primary Examiner

A. T. SURO PICÓ, Assistant Examiner

U.S. CL. X.R.

70 96-22, 114.7